

1

2,868,718

## PRECONDITIONING OF HYDROFORMING CATALYSTS

Walker F. Johnston, Jr., La Marque, Tex., assignor to  
The American Oil Company

No Drawing. Application November 29, 1954  
Serial No. 471,906

3 Claims. (Cl. 208—138)

This invention relates to the reforming of hydrocarbons. More particularly, it relates to the hydroforming of petroleum naphthas in the presence of an alumina-supported platinum catalyst.

One of the more successful techniques for upgrading petroleum naphthas employs a platinum-alumina catalyst at elevated temperature and pressure in the presence of added hydrogen. Such catalysts normally exhibit a more or less steady decline in activity, as evidenced by the octane number of the product, the rate of decline depending upon the process conditions, such as temperature, hydrogen partial pressure, charging stock composition, and the presence and proportions of deleterious substances such as sulfur, arsenic, nitrogen, and the like in the charging stock. The decline rate is especially rapid in the platinum hydroforming of the so-called naphthenic naphthas, i. e., naphthas containing more than 50 percent naphthenes and more than 70 percent naphthenes plus aromatics. An object of my invention is to precondition a platinum-alumina catalyst in such a way as to maintain its activity in the hydroforming of naphthenic naphthas. The observed deactivation tends to be emphasized at the high treating temperatures normally required to obtain premium gasolines of F-1 octane number of 90 or higher, making it correspondingly difficult to produce a reformate pool having an average octane number of the desired level. Another object of my invention is to extend the effective cycle length of platinum-alumina catalysts in the high-severity hydroforming of naphthenic naphthas. A further object is to increase the reformate pool octane number obtainable with platinum-alumina catalysts. These and other objects of my invention will be apparent from the appended description and claims.

My invention is basically a method for preconditioning a platinum-alumina catalyst to render it less susceptible to deactivation by naphthenic naphthas during the hydroforming thereof. In accordance with my invention, a platinum-alumina catalyst is subjected to a preliminary contact under hydroforming conditions for a period of 10 to 200 hours or more with a paraffinic naphtha, i. e., a naphtha containing more than about 30 percent paraffins and less than about 50 percent naphthenes. After the catalyst has been pretreated in this way, it is capable of maintaining its catalytic properties over an extended period in the hydroforming of a naphthenic naphtha, as hereinabove defined.

My new technique is applicable in the hydroforming of naphthenic naphthas to produce gasoline products having octane numbers of 90 to 100 or higher, and is especially adapted for the production of gasolines having octane numbers in the range of around 95 to 105. The hydroforming process is ordinarily carried out at a pressure within the range of about 100 to 1,000 pounds per square inch gage, a temperature between about 850 and 1,000° F., and hourly weight space velocity between about 0.5 and 5, and a hydrogen input rate between about 2,000

2

and 10,000 standard cubic feet per barrel of charging stock. For a product octane level above about 95, the pressure should preferably be between about 100 and 500 pounds per square inch gage, the temperature between about 925 and 975° F., and the space velocity between about 0.5 and 2. Under the foregoing conditions, it is commonly observed that the catalyst declines in activity at a rate greater than 2 F-1 octane numbers per 100 hours if the charging stock is a naphthenic naphtha.

In conditioning a platinum-alumina catalyst for contact with such a charging stock, I subject the catalyst to a preliminary treatment with a paraffinic naphtha, preferably having an ASTM final boiling point below about 425° F. and a sulfur content below about 0.05 weight percent, at a temperature between about 850 and 950° F., a pressure below about 500 pounds per square inch gage, and a weight hourly space velocity within the usual hydroforming range of about 0.5 to 5 for a period of around 10 hours or more. I prefer to carry out the pretreatment for a sufficient length of time to reach a substantially constant catalyst activity decline rate, operating under the hydroforming conditions thereafter to be employed, and for this purpose a pretreating time of around 25 to 100 hours is ordinarily sufficient, depending upon the refractoriness of the stock employed in the pretreatment.

By the foregoing means, I have succeeded in effecting a large decrease in the activity decline rates of platinum-alumina catalysts when employed for the hydroforming of naphthenic charging stocks. After catalysts have been treated in this way, I find that they commonly exhibit an activity decline rate less than 1 F-1 octane number per 100 hours in the ensuing hydroforming operation.

The extent of improvement in each case depends upon the degree of pretreatment and upon the severity of deactivation ordinarily produced by the naphthenic stock. The effectiveness of my new technique is conveniently illustrated in connection with the hydroforming of a Texas City naphthenic heavy naphtha, containing around 60 percent naphthenes and around 80 percent naphthenes plus aromatics. Such a naphtha, when hydroformed under substantially isothermal conditions at 920° F., 300 pounds per square inch gage, 1.5 weight hourly space velocity, and 5,000 standard cubic feet of hydrogen per barrel, ordinarily exhibits an octane decline rate of 10 F-1 units per 100 hours. When the catalyst is subjected to a pretreatment for 10 to 100 hours or more under the same conditions with a Texas City paraffinic heavy naphtha containing around 40 percent of paraffins, the decline rate in the subsequent hydroforming of the naphthenic heavy naphtha is reduced to less than 1 F-1 unit per 100 hours.

I am uncertain as to the precise mechanism whereby the advantageous results of my preconditioning operation are achieved. My technique is not an equivalent of rerunning, acid treating, clay treating, silica-gel treating, or any of the other methods commonly employed for removing contaminants from petroleum stocks, since such methods do not produce the improved catalyst activity maintenance typical of my invention. It seems likely, in fact, that the removal of catalyst poisons is not involved, since I have successfully employed a paraffinic naphtha pretreating stock which was somewhat higher in sulfur content than the naphthenic naphtha subsequently processed. Whatever its method of action, however, my pretreating step is effective in prolonging the useful cycle life of platinum-alumina catalysts.

My invention will be more fully understood from the following operating examples:

## Example 1

A Texas City naphthenic heavy naphtha having an ASTM boiling range of 258 to 402° F. and an API gravity of 45.7°, and containing 20 volume-percent paraffins, 58 percent naphthenes, 22 percent aromatics, 0.015 weight-percent sulfur, and 7 parts per million nitrogen, was subjected to hydroforming under isothermal conditions in the presence of a 0.6 percent platinum-on-alumina catalyst at 923° F., 300 pounds per square inch gage, 1.5 hourly weight space velocity, and 5,000 standard cubic feet of added hydrogen per barrel. The resulting data showed an activity decline rate of 10 F-1 units per 100 hours on stream.

In a comparative test, the catalyst was pretreated for 216 hours under the same conditions with a Texas City paraffinic heavy naphtha having a boiling range of 222 to 406° F. and an API gravity of 50.7°, and containing 38 volume-percent paraffins, 1 percent olefins, 48 percent naphthenes, 13 percent aromatics, 0.035 weight-percent sulfur, and approximately 7 parts per million of nitrogen. At the end of this time, the flow of paraffinic naphtha was discontinued and the naphthenic naphtha was introduced and treated under the same process conditions. The reformate F-1 octane rating decreased from 100.9 to 99.4 during the next 300 hours, corresponding to an activity decline rate of only 0.5 F-1 unit per 100 hours on stream.

## Example 2

A Texas City paraffinic heavy naphtha having a final boiling point of 437° F. and containing 38 percent paraffins, 1 percent olefins, 48 percent naphthenes, and 13 percent aromatics, by volume, was subjected to reforming in the presence of a 0.6 percent platinum-on-alumina catalyst at 300 pounds per square inch gage, 1.0 hourly weight space velocity, 927° F., and 5,000 standard cubic feet of hydrogen per barrel. The initial F-1 octane number was 100.1 and the catalyst activity decline rate was 1.2 F-1 units per 100 hours. At the end of 136 hours on stream, the charging stock was changed to a Texas City paraffinic heavy naphtha having a final boiling point of 442° F. No marked difference in results was noted between the two naphthas.

At the end of 184 hours on the paraffinic naphthas, the charging stock was changed to a Texas City naphthenic heavy naphtha having an ASTM final boiling point of 404° F. and containing 20 percent paraffins, 58 percent naphthenes, and 22 percent aromatics, by volume, together with 0.015 weight-percent sulfur. The hydroforming was continued under the same conditions, and a product was obtained during the 216-232 hour period having an F-1 octane level of 101.3. The reformate octane number declined to 99.6 during the 376-392 hour period, corresponding to a decline rate of about 1.0 F-1 unit per 100 hours.

My new process is effective for preconditioning alumina-supported platinum hydroforming catalysts in general, many types of which have been described in the prior art. It can be used, for example, in connection with unpromoted platinum-on-alumina, or with platinum-alumina catalysts which include a promoting additive such as vanadia, chromia, titania, iridium, an oxide of phosphorus, or the like, or a mild cracking adjuvant, such as boria, silica, fluorine, chlorine, or the like. The catalysts commonly contain platinum in a proportion between about 0.05 and 1 percent by weight, based on dry  $Al_2O_3$ . Promoters and other additives are usually employed in a proportion between about 0.1 and 8 percent by weight.

While I have described my invention with reference to certain specific embodiments thereof, it is to be understood that such embodiments are illustrative only and not by way of limitation. Numerous alternative charging stocks, catalysts, manipulative steps, and operating

conditions will be apparent from the above description to those skilled in the art.

In accordance with the foregoing description, I claim as my invention:

1. In a method for hydroforming a naphthenic petroleum naphtha containing above about 50 percent naphthenes and above about 70 percent naphthenes and aromatics in the presence of an alumina-supported platinum catalyst at a hydroforming temperature between about 850 and 1000° F. and obtaining therefrom a gasoline having an F-1 octane number above about 90, in which operation the activity of said catalyst ordinarily declines at a rate greater than about 2 F-1 units per 100 hours, the improvement which comprises preconditioning said catalyst prior to said hydroforming operation by exposing said catalyst when fully active to contact under hydroforming conditions with a paraffinic petroleum naphtha containing above about 30 percent paraffins and less than about 50 percent naphthenes for a period of time between about 10 and 200 hours, whereby the rate of decline in activity of the said catalyst in the ensuing hydroforming operation is reduced to less than about 1 F-1 octane unit per 100 hours.

2. In a method for hydroforming a naphthenic petroleum naphtha containing above about 50 percent naphthenes and above about 70 percent naphthenes and aromatics in the presence of an alumina-supported platinum catalyst at a hydroforming temperature between about 850 and 1000° F. and a pressure between about 100 and 500 pounds per square inch gage and obtaining therefrom a gasoline having an F-1 octane number between about 95 and 105, in which operation the activity of said catalyst ordinarily declines at a rate greater than about 2 F-1 units per 100 hours, the improvement which comprises preconditioning said catalyst prior to said hydroforming operation by exposing said catalyst when fully active to contact under hydroforming conditions with a paraffinic petroleum naphtha containing above about 30 percent paraffins and less than about 50 percent naphthenes for a period of time between about 10 and 200 hours, whereby the rate of decline in activity of said catalyst in the ensuing hydroforming operation is reduced to less than about 1 F-1 octane unit per 100 hours.

3. In a method for hydroforming a naphthenic petroleum naphtha containing above about 50 percent naphthenes and above about 70 percent naphthenes and aromatics in the presence of a fixed-bed catalyst consisting essentially of alumina and between about 0.05 and 1 percent by weight of platinum, based on dry  $Al_2O_3$ , at a pressure between about 100 and 500 pounds per square inch gage and a hydroforming temperature between about 850 and 1000° F. sufficient to obtain therefrom a gasoline having an F-1 octane number between about 95 and 105, whereby the activity of said catalyst ordinarily declines at a rate greater than about 2 F-1 octane units per 100 hours, the improvement which comprises preconditioning said catalyst prior to said hydroforming operation by exposing said catalyst when fully active for a period of between about 25 and 100 hours to contact under hydroforming conditions with a paraffinic petroleum naphtha containing above about 30 percent paraffins, less than about 50 percent naphthenes, and less than about 0.05 percent sulfur, whereby the rate of decline in activity of said catalyst in the ensuing hydroforming operation is reduced to less than about 1 F-1 octane unit per 100 hours.

## References Cited in the file of this patent

## UNITED STATES PATENTS

2,689,208 Murray et al. Sept. 14, 1954  
2,723,946 Donaldson Nov. 15, 1955

## OTHER REFERENCES

"Chemical Constituents of Petroleum," by Sachanen, page 199 (1945), Reinhold Pub. Co., New York, N. Y.